



US005276239A

**United States Patent** [19]

Sanderson John R. et al.

[11] **Patent Number:** **5,276,239**[45] **Date of Patent:** **Jan. 4, 1994**

[54] **DIMERIZATION OF LONG-CHAIN OLEFINS USING A SILICA GEL ALKYSULFONIC ACID**

[75] Inventors: **Sanderson John R., Leander; John F. Knifton, Austin; Edward T. Marquis, Austin, all of Tex.**

[73] Assignee: **Texaco Chemical Company, White Plains, N.Y.**

[21] Appl. No.: **919,455**

[22] Filed: **Jul. 27, 1992**

[51] Int. Cl.<sup>5</sup> ..... **C07C 2/26; C07C 2/34**

[52] U.S. Cl. ..... **585/511; 585/510; 585/515**

[58] Field of Search ..... **585/510, 511, 515**

[56] **References Cited**

**U.S. PATENT DOCUMENTS**

|           |         |                |
|-----------|---------|----------------|
| 2,593,417 | 4/1952  | D'Alelio       |
| 2,834,819 | 5/1958  | D'Alelio       |
| 3,149,178 | 9/1964  | Hamilton       |
| 3,742,082 | 6/1973  | Brennan        |
| 4,022,847 | 5/1977  | McClure        |
| 4,038,213 | 7/1977  | McClure et al. |
| 4,056,578 | 11/1977 | McClure et al. |
| 4,060,565 | 11/1977 | McClure et al. |
| 4,065,512 | 12/1977 | Cares          |
| 4,065,515 | 12/1977 | McClure et al. |
| 4,180,695 | 12/1979 | McClure        |
| 4,400,565 | 8/1983  | Darden et al.  |
| 4,613,723 | 9/1986  | Olah           |
|           |         | 585/730        |
|           |         | 585/10         |
|           |         | 585/730        |

4,683,216 7/1987 Farcasieu ..... 502/159  
4,837,372 6/1989 Zimmerman ..... 585/514  
4,912,280 3/1990 Clerici ..... 585/516

**OTHER PUBLICATIONS**

R. D. Badley and W. T. Ford, "Silica-Bound Sulfonic Acid Catalysts", *J. Org. Chem.*, 1989, 54, pp. 5437-5443.

"Catalytic Uses of Nafion Perfluorosulfonic Acid Products", Research Disclosure Jul. 1980 No. 195.

J. D. Weaver et al., "Supported Fluoro-carbonsulfonic Acid Polymer Heterogenous Acid Catalyst," *Catalysis* 1987, pp. 483-489.

Rajadhyaksha and Chaudari, "Alkylation of Phenol and Pyrocatechal by Isobutyl Using Superacid Catalysts," *Ind. Eng. Res.*, 26 1276-1280 (1987).

*Primary Examiner*—Patrick P. Garvin

*Assistant Examiner*—E. D. Irzinski

*Attorney, Agent, or Firm*—James L. Bailey; Kenneth R. Priem; Russell R. Stolle

[57] **ABSTRACT**

A process is disclosed for preparing synthetic lubricant base stocks having a high dimer to trimer ratio from long-chain olefins. These synthetic lubricant base stocks are prepared in good yield by dimerizing linear olefins using a catalyst comprising a silica gel alkylsulfonic acid.

**15 Claims, No Drawings**

**DIMERIZATION OF LONG-CHAIN OLEFINS  
USING A SILICA GEL ALKYSULFONIC ACID**

**CROSS-REFERENCE TO RELATED  
APPLICATION**

This application is related to allowed U.S. patent application Ser. No. 07/597,267, filed Oct. 15, 1990, and issued Mar. 17, 1992, as U.S. Pat. No. 5,097,087.

**BACKGROUND OF THE INVENTION**

**1. Field of the Invention**

The invention relates to the preparation of synthetic lubricant base stocks, and more particularly to synthetic lubricant base stocks made by dimerizing long-chain linear olefins.

**2. Description of Related Methods**

Synthetic lubricants are prepared from man-made base stocks having uniform molecular structures and, therefore, well-defined properties that can be tailored to specific applications. Mineral oil base stocks, on the other hand, are prepared from crude oil and consist of complex mixtures of naturally occurring hydrocarbons. The higher degree of uniformity found in synthetic lubricants generally results in superior performance properties. For example, synthetic lubricants are characterized by excellent thermal stability. As automobile engines are reduced in size to save weight and fuel, they run at higher temperatures, therefore requiring a more thermally stable oil. Because lubricants made from synthetic base stocks have such properties as excellent oxidative/thermal stability, very low volatility, and good viscosity indices over a wide range of temperatures, they offer better lubrication and permit longer drain intervals, with less oil vaporization loss between oil changes.

Generally, synthetic base stocks are prepared by oligomerizing internal and alpha-olefin monomers to form a mixture of dimers, trimers, tetramers, and pentamers, with minimal amounts of higher oligomers. The unsaturated oligomer products are then hydrogenated to improve their oxidative stability. The resulting synthetic base stocks have uniform isoparaffinic hydrocarbon structures similar to high quality paraffinic mineral base stocks, but have the superior properties mentioned due to their higher degree of uniformity.

Synthetic base stocks are produced in a broad range of viscosity grades. It is common practice to classify the base stocks by their viscosities, measured in centistokes (cSt) at 100° C. Those base stocks with viscosities less than or equal to about 4 cSt are commonly referred to as "low viscosity" base stocks, whereas base stocks having a viscosity in the range of around 40 to 100 cSt are commonly referred to as "high viscosity" base stocks. Base stocks having a viscosity of about 4 to about 8 cSt are referred to as "medium viscosity" base stocks. The low viscosity base stocks generally are recommended for low temperature applications. Higher temperature applications, such as motor oils, automatic transmission fluids, turbine lubricants, and other industrial lubricants, generally require higher viscosities, such as those provided by medium viscosity base stocks (i.e. 4 to 8 cSt grades). High viscosity base stocks are used in gear oils and as blending stocks.

The viscosity of the base stocks is determined by the length of the oligomer molecules formed during the oligomerization reaction. The degree of oligomerization is affected by the catalyst and reaction conditions

employed during the oligomerization reaction. The length of the carbon chain of the monomer starting material also has a direct influence on the properties of the oligomer products. Fluids prepared from short-chain monomers tend to have low pour points and moderately low viscosity indices, whereas fluids prepared from long-chain monomers tend to have moderately low pour points and higher viscosity indices. Oligomers prepared from long-chain monomers generally are more suitable than those prepared from shorter-chain monomers for use as medium viscosity synthetic lubricant base stocks.

One known approach to oligomerizing long-chain olefins to prepare synthetic lubricant base stocks is to contact the olefin with boron trifluoride together with a promotor at a reaction temperature sufficient to effect oligomerization of the olefin. See, for example, co-assigned U.S. Pat. Nos. 4,400,565; 4,420,646; 4,420,647; and 4,434,308. However, boron trifluoride gas (BF<sub>3</sub>) is a pulmonary irritant, and breathing the gas or fumes formed by hydration of the gas with atmospheric moisture poses hazards preferably avoided. Additionally, for some applications, such as semi-synthetic oils or where low temperature properties are important, a higher dimer to trimer ratio than that obtained using such conventional oligomerization catalysts is desirable.

A method for dimerizing long-chain olefins using a less hazardous catalyst is taught in co-assigned U. S. Pat. No. 4,367,352 to Watts, Jr. et al., which discloses the use of a perfluorosulfonic acid resin to dimerize long-chain alpha-olefins. At column 3, the '352 patent teaches that the perfluorosulfonic acid resin produces a high dimer to trimer ratio, and gives an example showing percent dimer and percent trimer in a ratio of about 4.77:1. Applicants have discovered, surprisingly, that a substantially higher dimer/trimer ratio may be obtained by contacting the olefin feed with a catalyst comprising a silica gel alkylsulfonic acid. Like the resins of the '352 Patent, the silica gel alkylsulfonic acids also are less hazardous and more easily handled than boron trifluoride. Applicants believe it was heretofore unknown in the art to use silica gel alkylsulfonic acids to prepare synthetic lubricant base stocks having a very high percentage of dimers. By maintaining a low percentage of trimer and higher oligomers in the reaction product, Applicants are able to obtain base stocks having excellent low temperature properties while using long-chain monomers as feedstock.

**SUMMARY OF THE INVENTION**

The invention relates to a process for the preparation of synthetic lubricant base stocks having a high dimer to trimer ratio, comprising contacting linear olefins containing from 10 to 24 carbon atoms with a heterogenous catalyst comprising a silica gel alkylsulfonic acid, wherein the olefins are contacted with the catalyst at a temperature of from about 50° C. to about 300° C. The invention further relates to a process for the preparation of synthetic lubricant base stocks having a high dimer to trimer ratio, comprising contacting linear olefins containing from 14 to 24 carbon atoms with a silica gel alkylsulfonic acid catalyst having the following structure:



wherein R is an alkyl group having from 1 to 3 carbon atoms and n is an integer in the range of 3 to 10, and recovering a bottoms product having a dimer to trimer ratio of about 5:1 or greater.

#### DESCRIPTION OF THE PREFERRED EMBODIMENTS

The olefin monomer feed stocks used in the present invention may be selected from compounds comprising (1) alphaolefins having the formula  $\text{R}''\text{CH}=\text{CH}_2$ , where  $\text{R}''$  is an alkyl radical of 8 to 22 carbon atoms, and (2) internal olefins having the formula  $\text{RCH}=\text{CHR}'$ , where R and R' are the same or different alkyl radicals of 1 to 21 carbon atoms, provided that the total number of carbon atoms in any one olefin shall be within the range of 10 to 24, inclusive. A preferred range for the total number of carbon atoms in any one olefin molecule is 14 to 18, inclusive, with an especially preferred range being 14 to 16, inclusive. Mixtures of internal and alphaolefins may be used, as well as mixtures of olefins having different numbers of carbon atoms, provided that the total number of carbon atoms in any one olefin shall be within the range of 10 to 24, inclusive. The alpha and internal-olefins to be dimerized in this invention may be obtained by processes well-known to those skilled in the art and are commercially available.

When the olefin feed contacts the catalyst several reactions may occur. Initially, olefin monomer reacts with olefin monomer to form dimers. The dimerization reaction may be represented by the following general equation:



where m represents the number of carbon atoms in the monomer. Some of the dimers that are formed then react with additional olefin monomer to form trimers, and so on, though to a much more limited extent than is observed using prior art catalysts. Thus are Applicants able to obtain base stocks with a substantially higher dimer to trimer ratio than may be obtained with prior art catalysts. Generally, each resulting dimer or higher oligomer contains one double bond.

The catalysts used to effect this reaction are silica gel alkylsulfonic acids. As used in this application, the term "silica gel alkylsulfonic acids" means silica having alkylsulfonic acid groups chemically bound thereto. In other words, the alkylsulfonic acids are not merely deposited on the silica, but covalently bonded to the silica. Other catalysts within the scope of the present inventive process include alkylsulfonic acids bound to other Group IV oxides, such as titania, zirconia, and the like, or bound to Group III oxides, such as alumina, and the like.

Preferably, the silica gel alkylsulfonic acids used in the present invention have the following structure:



wherein R is an alkyl group having from 1 to 3 carbon atoms and n is an integer in the range of 3 to 10. More preferably, the silica gel alkylsulfonic acid used in the present invention is silica gel propylsulfonic acid. The preparation of silica-bound sulfonic acids is exemplified herein by the preparation of silica gel propylsulfonic acid.

Silica gels are commercially available in at least the following mesh sizes: 3-8; 6-16; 14-20; 14-42; and 28-200 and greater. A suitable commercially available silica gel is the grade 12, 28-200 mesh, silica gel available from Aldrich Chemical Co., Inc. Silica gel propylsulfonic acid may be prepared by treating silica gel with (3-mercaptopropyl)trimethoxysilane. The resulting surface-modified mercaptan is then oxidized using aqueous  $\text{H}_2\text{O}_2$ , to give the silica-bound sulfonic acid.



45 This and other procedures are more fully described by R. D. Badley and W. T. Ford, in "Silica-Bound Sulfonic Acid Catalysts", *J. Org. Chem.*, vol. 54, no. 23, pages 5437-5443 (1989), incorporated herein by reference, and in the Examples of this application.

50 The dimerization reaction may be carried out in either a stirred slurry reactor or in a fixed bed continuous flow reactor. The catalyst concentration should be sufficient to provide the desired catalytic effect. The temperatures at which the dimerization may be performed 55 are between about 50° and 300° C., with the preferred range being from about 140° to about 180° C. It is especially preferred that the temperature be about 140° to about 160° C.

At reaction temperatures of about 200° C. or greater, 60 the amount of unsaturation remaining in the products of the oligomerization reaction may decrease, thus reducing the degree of hydrogenation necessary to remove unsaturation from the base stocks. However, temperatures above 200° C. may adversely affect olefin conversion and the dimer to trimer ratio. Applicants have found that the addition of a hydrocarbon containing a tertiary hydrogen, such as methylcyclohexane, may further reduce the amount of unsaturation present in the

base stocks. One skilled in the art may choose the reaction conditions most suited to the results desired for a particular application. The reaction may be run at pressures of from 0 to 1000 psig.

Following the dimerization reaction, the unsaturated dimers, and any higher oligomers present, may be hydrogenated to improve their thermal stability and to guard against oxidative degradation during their use as lubricants. Hydrogenation processes known to those skilled in the art may be used to hydrogenate the dimer-rich bottoms. A number of metal catalysts are suitable for promoting the hydrogenation reaction, including nickel, platinum, palladium, copper, and Raney nickel. These metals may be supported on a variety of porous materials such as kieselguhr, alumina, or charcoal, or they may be formulated into a bulk metal catalyst. A particularly preferred catalyst for this hydrogenation is a nickel-copper-chromia catalyst described in U.S. Pat. No. 3,152,998, incorporated by reference herein. Other U.S. patents disclosing known hydrogenation procedures include U.S. Pat. Nos. 4,045,508; 4,013,736; 3,997,622; and 3,997,621.

Unreacted monomer may be removed either prior to or after the hydrogenation step. Optionally, unreacted monomer may be stripped from the reaction products prior to hydrogenation and recycled to the catalyst bed for dimerization. The removal or recycle of unreacted monomer or, if after hydrogenation, the removal of non-dimerized alkane, should be conducted under mild conditions using vacuum distillation procedures known to those skilled in the art. Distillation at temperatures exceeding 250° C. may cause the dimers to break down in some fashion and come off as volatiles. Preferably, therefore, the reboiler or pot temperature should be kept at 0 under about 225° C. when stripping out the monomer. Procedures known by those skilled in the art to be alternatives to vacuum distillation also may be employed to separate unreacted components from the dimer-rich bottoms product.

While it is known to include a distillation step after the hydrogenation procedure to obtain products of various 100° C. viscosities, it is preferred in the method of the present invention that no further distillation (beyond monomer flashing) be conducted. In other words, the monomer-stripped, hydrogenated bottoms are the desired synthetic lubricant components. Thus, the method of this invention does not require the costly, customary distillation step, yet, surprisingly, produces a synthetic lubricant component that has excellent properties and that performs in a superior fashion. However,

in some contexts, one skilled in the art may find subsequent distillation useful in the practice of this invention.

The invention will be further illustrated by the following examples, which are given by way of illustration and not as limitations on the scope of this invention. The entire text of every patent, patent application or other reference mentioned above is hereby incorporated herein by reference.

## EXAMPLES

In the examples detailed below, the following procedure was used:

### Catalyst Preparation

15 Silica gel (500 g) and 10% HCl (1000 g) were refluxed for 4.0 hours. The solid was collected with suction and washed with water until the washings were neutral to litmus. The solid was then dried at 100° C. in a vacuum oven overnight.

20 500 g of the above silica gel was treated with 1000 g of toluene and refluxed for 5.0 hours. (A Dean-Stark trap was used to remove the small amount of water remaining.) The trap was removed and 125 g of (3-mercaptopropyl) trimethoxysilane was added. The mixture was refluxed for 25 to 30 hours, and then cooled to ambient temperature. The solid was collected with suction and washed with toluene followed by acetone. The solid was dried in a vacuum oven at 100° C. overnight.

25 To 500 g of the mercaptopropyl silica gel from above was slowly added 400 g water and 1500 g 30% hydrogen peroxide. The slurry was stirred slowly overnight, and then let stand over the weekend. The solid was then collected with suction and washed with water and acetone, toluene, and then acetone once more. Finally the solid was dried in a vacuum oven overnight at 100° C. The dried material had the following analysis.

|          |           |
|----------|-----------|
| Acidity: | 20.2 mg/g |
| Sulfur:  | 1.7%      |
| Water:   | 0.82%     |

### Olefin Oligomerization

45 Olefin and catalyst were charged to a flask equipped with a stirrer, thermometer, heating mantle, condenser, and nitrogen purge. The mixture was heated to the desired temperature, for the desired time, with vigorous stirring. At the end of the reaction, the mixture was cooled to ambient temperature, filtered with suction, and the liquid effluent analyzed by liquid chromatography. The results are shown in the table below.

| Ex. No. | Catalyst | Oligomerization of Olefins Using Silica Gel Propyl Sulfonic Acid |               |            |           |          |             |      |
|---------|----------|------------------------------------------------------------------|---------------|------------|-----------|----------|-------------|------|
|         |          | (g) of Catalyst                                                  | (g) of Olefin | Temp (°C.) | Time (Hr) | Con. (%) | D/T + Ratio |      |
| 1       | SGPSA    | 10                                                               | 10 $\alpha$   | 100        | 160       | 5.0      | 54.4        | 5.98 |
| 2       | SGPSA    | 10                                                               | 10 $\alpha$   | 100        | 180       | 4.0      | 30.5        | 5.10 |
| 3       | SGPSA    | 10                                                               | 10 $\alpha$   | 100        | 120       | 6.0      | 16.6        | —    |
| 4       | SGPSA    | 10                                                               | 10 $\alpha$   | 100        | 140       | 6.0      | 45.4        | 9.83 |
| 5       | SGPSA    | 10                                                               | 10 $\alpha$   | 100        | 160       | 5.0      | 57.3        | 7.05 |
| 6       | SGPSA    | 5                                                                | 10 $\alpha$   | 100        | 160       | 5.0      | 25.3        | 6.19 |
| 7       | SGPSA    | 20                                                               | 10 $\alpha$   | 100        | 160       | 5.0      | 82.4        | 3.40 |
| 8       | SGPSA    | 10                                                               | 1314 I        | 100        | 160       | 5.0      | 31.0        | 5.99 |
| 9       | SGPSA    | 10                                                               | 14 $\alpha$   | 100        | 160       | 5.0      | 31.8        | 6.95 |
| 10      | SGPSA    | 10                                                               | 1416 $\alpha$ | 100        | 160       | 5.0      | 40.6        | 9.63 |
| 11      | SGPSA    | 10                                                               | 1518 I        | 100        | 160       | 5.0      | 25.6        | —    |

-continued

| Oligomerization of Olefins Using Silica Gel Propyl Sulfonic Acid |          |                 |               |            |           |                      |
|------------------------------------------------------------------|----------|-----------------|---------------|------------|-----------|----------------------|
| Ex. No.                                                          | Catalyst | (g) of Catalyst | (g) of Olefin | Temp (°C.) | Time (Hr) | Con. (%) D/T + Ratio |
| 12                                                               | None     | 10              | 10 $\alpha$   | 100        | 160       | 5.0 0.00             |

SGPSA = Silica gel propylsulfonic acid;

Con. = olefin conversion;

D/T + Ratio = ratio of dimer to trimer;

I = internal olefin;

 $\alpha$  = alpha olefin.

We claim:

1. A process for the preparation of synthetic lubricant base stocks, comprising contacting linear olefins containing from 10 to 24 carbon atoms with a heterogenous catalyst comprising a silica gel alkylsulfonic acid having the following structure:



wherein the alkylsulfonic acid in said structure is covalently bonded to the silica gel and R is an alkyl group having from 1 to 3 carbon atoms and n is an integer in the range of 3 to 10, and wherein the olefins are contacted with the catalyst at a temperature of from about 50° C. to about 300° C.

2. The process of claim 1, wherein the linear olefins contain from 14 to 18 carbon atoms.

3. The process of claim 1, wherein the linear olefins contain from 14 to 16 carbon atoms.

4. The process of claim 1, wherein the olefins are contacted with the catalyst at a temperature of about 140° C. to about 160° C.

5. A process for the preparation of synthetic lubricant base stocks, comprising contacting linear olefins containing from 14 to 24 carbon atoms with a heterogenous catalyst comprising a silica gel alkylsulfonic acid having the following structure:



wherein the alkylsulfonic acid is covalently bonded to the silica gel and R is an alkyl group having from 1 to 3 carbon atoms and n is an integer in the range of 3 to 10, and wherein the olefins are contacted with the catalyst at a temperature of from about 50° C. to about 300° C.

and recovering a bottoms product having a dimer to trimer ratio of about 5:1 or greater.

6. The process of claim 5, wherein the linear olefins contain from 14 to 18 carbon atoms.

7. The process of claim 5, wherein the linear olefins contain from 14 to 16 carbon atoms.

8. The process of claim 5, wherein the olefins are contacted with the catalyst at a temperature of about 140° C. to about 160° C.

9. The process of claim 5, wherein the olefins are contacted with the catalyst at a temperature of about 140° C. and the base stock recovered has a dimer to trimer ratio of about 9:1 or greater.

10. A process for the preparation of a synthetic lubricant base stock, comprising the following steps: (a) contacting linear olefins containing from 14 to 24 carbon atoms with a catalyst comprising a silica gel propylsulfonic acid polymer having the following structure:



wherein the propylsulfonic acid is covalently bonded to the silica gel and R is an alkyl group having from 1 to 3 carbon atoms, and wherein the catalyst and olefin are contacted at a temperature of about 140° C. to about 160° C.; (b) separating out any remaining un-reacted olefins to recover a synthetic lubricant base stock having a dimer to trimer ratio of about 5:1 or greater; and (c) hydrogenating the base stock resulting from step (b).

11. The process of claim 10, wherein the linear olefins contain from 14 to 18 carbon atoms.

12. The process of claim 10, wherein the linear olefins contain from 14 to 16 carbon atoms.

13. The process of claim 10, wherein the olefins are contacted with the catalyst at a temperature of about 140° C.

14. The process of claim 10, wherein the olefins are contacted with the catalyst at a temperature of about 140° C. and the base stock recovered has a dimer to trimer ratio of about 9:1 or greater.

15. The process of claim 10, wherein R is methyl group.

\* \* \* \* \*